

1

3,336,158  
METHOD OF RENDERING ARTICLES  
WATER-REPELLENT

Nobuaki Wada, Ibaraki-shi, Kazumune Nakao, Higashisumiyoshi-ku, Osaka-shi, Toshiya Tsuji, Yao-shi, Osaka-fu, and Mitsuji Shibata, Fushimi-ku, Kyoto-shi, Japan, assignors to The Governor of Osaka-fu, and to Nihon Mengyo Gijutsu Kenkyuso, a foundation of Japan, both of Osaka-shi, Japan

No Drawing. Filed Feb. 28, 1964, Ser. No. 348,280  
6 Claims. (Cl. 117—161)

This invention relates to the method of rendering articles water-repellent. More particularly, the invention pertains to a novel method of rendering articles water-repellent, comprising applying a polysiloxane having a methylhydrogensiloxane unit, such as methylhydrogenpolysiloxane.

Methylhydrogenpolysiloxane is known in the art as a silicon water-repelling agent. In order to produce in a single application satisfactory water-repellent effects, the articles treated with said agent are normally baked or cured at a temperature higher than 150° C., but the resultant wash durability and dry-cleaning resistance are not always satisfactory.

In the prior art, there is accordingly employed a catalyst, such as zinc or stannous 2-ethylhexanoate, zirconium oxychloride, zinc acetate, sodium bicarbonate and the like. The application of said catalyst, however, does not necessarily exclude the necessity of baking or curing at a high temperature, and the resultant effects are confined to improvements in the wash durability and the like qualities of the treated articles. The application of said method, moreover, is restricted to the treatment of nylon, polyester, cellulose acetate and the like hydrophobic fibers and fabrics, producing almost no marked durability in cotton, linen viscose rayon stable, polyvinyl alcohol and the like hydrophilic fibers and fabrics, and the resultant water-repellency is markedly deteriorated even by a single washing. Consequently, the prior art in general can hardly be applied to the articles having poor heat resistance.

There is disclosed in the United States Patent 2,588,365 a method comprising applying a mixture of methylhydrogenpolysiloxane and dimethylpolysiloxane at a temperature ranging from 100° to 475° F. However, it remains also impracticable for said patent to achieve the desired water-repellency without subjecting the wetted articles to a heat processing in order to thermally decompose the emulsifier, insofar as said mixture is employed in the form of emulsion.

The primary object of the present invention is accordingly to provide a method for rendering articles water-repellent which can be applied without subjecting the wetted articles to heat processing, such as baking or curing.

Another object of the present invention is to provide a method for rendering articles water-repellent, wherein the drying of the treated articles can be carried out at room temperature, producing a marked water-repellency.

A further object of the present invention is to provide a method for rendering articles water-repellent, wherein the wash durability, resistance to dry cleaning, and other properties of the resultant articles can be markedly improved.

A still further object of the present invention is to provide a method for rendering articles water-repellent, which can be applied not only to the hydrophobic fibers and fabrics but to cotton, rayon, staple, polyvinyl alcohol and the like hydrophilic fibers and fabrics, producing a marked durability, dry-cleaning resistance and the like desirable effects.

2

The present invention is based upon the discovery that a metallic compound applied in a small quantity in admixture with a catalyst, such as zinc acetate or zinc formate, which is employed in association with a polysiloxane having a methylhydrogensiloxane unit in the order of at least 50 weight percent, produces marked effects which cannot be achieved by the single application of said catalyst, rendering it completely possible to carry out the dry processing of the resultant articles at room temperature, and imparting a marked water-repellency and durability not only to the hydrophobic but to the hydrophilic fibers and fabrics as well.

The polysiloxanes employed as a water-repelling agent in the present invention are methylhydrogenpolysiloxane, copolymers of methylhydrogendifchlorosiloxane and dimethylchlorosilane, mixtures of methylhydrogenpolysiloxane and dimethylpolysiloxane and the like materials having a methylhydrogensiloxane unit in the order of more than 50 weight percent. The resultant water-repellency can be increased with a rise in the number of said unit present in the materials employed.

In the present invention, any of the aforespecified polysiloxanes is employed by emulsifying in a concentration of from 1 to 10 weight percent. Particularly desirable results are obtained with a concentration of about 3 weight percent.

The emulsifying agent employed in the present invention are cationic emulsifiers, such as quaternary ammonium salt; anionic emulsifiers, such as dialkyl ester of succinic sulfonate, alkylbenzene sulfonate and aliphatic acid soaps; and nonionic emulsifiers, such as polyoxyethylene sorbitanmonolaurate and polyoxyethylene sorbitanmonoolate. The most desirable effects are obtained with cationic emulsifiers, particularly with quaternary ammonium salt.

In the present invention, there is employed zinc acetate in admixture with at least one species of metallic compounds, such as zirconyl acetate, tin acetate, magnesium acetate, zinc salts of higher aliphatic acids having from 8 to 18 carbon atoms, sodium salts of higher aliphatic acids having from 8 to 18 carbon atoms, zirconium oxychloride, zinc oxide, titanium oxide, tin oxide and lead oxide. Zinc formate can also be used in the place of zinc acetate, producing the same results as zinc acetate does.

In the present invention, the desired effects can be obtained when any of the aforespecified metallic compounds is employed singly or in admixture in a very small metal weight in relation to the zinc weight of the aforesaid catalyst. In the following table are shown the desirable weight range of application, wherein the metal weight of each metallic compound is determined in terms of the zinc weight of zinc acetate or zinc formate as 1, and in which the value is on the average because the value fluctuates in accordance with the articles to be treated and the emulsifier to be employed:

| Metallic Compounds         | Desirable Range of Application | Most Desirable Range of Application |
|----------------------------|--------------------------------|-------------------------------------|
| Zirconyl acetate.....      | 1/1,000-1/10                   | 1/100                               |
| Tin acetate.....           | 1/100-1/10                     | 5/100                               |
| Magnesium acetate.....     | 1/10-1/2                       | 2/10-3/10                           |
| Zinc stearate.....         | 1/1,000-3/10                   | 1/100-1/10                          |
| Zirconium oxychloride..... | 1/1,000-1/10                   | 1/100-1/10                          |
| Zinc oxide.....            | 1/100-7/10                     | 1/10-5/10                           |
| Titanium oxide.....        | 1/100-7/10                     | 1/10-5/10                           |
| Tin oxide.....             | 1/100-7/10                     | 1/10-5/10                           |
| Lead oxide.....            | 1/100-7/10                     | 1/10-5/10                           |

In the present invention, any of the aforespecified metallic compounds and zinc acetate or zinc formate are employed in the order of from 1 to 15 percent, preferably from 8 to 12 percent, by total metal weight in relation

to the polysiloxane employed. Particularly desirable results are obtained when said metallic compound and zinc acetate or zinc formate are employed in the order of about 10 percent by total metal weight.

The articles which can be treated according to the principles of the present invention include not only nylon, polyester, cellulose acetate, polyacrylonitrile and copolymers of acrylonitrile, all in the form of fibers, fabrics and fabricated articles, but cotton, linen, viscose rayon staple, polyvinyl alcohol and other hydrophilic synthetic fibers, fabrics and fabricated articles. Articles of paper, wood, glass, concrete and metals can also be treated according to the principles of the present invention, producing a marked extent of water-repellency.

In actual operation, any of the aforespecified metallic compounds is added in association with zinc acetate or zinc formate to the emulsion containing any of the aforespecified polysiloxanes. The article to be treated is wetted with the resultant emulsion by a suitable method, such as dipping, coating, spraying or the like, and allowed to dry at room temperature, namely from 10° to 40° C. or thereabout, for a day or two. The period of time required for drying the wetted articles is dependent upon the species of the emulsifier and the metallic compound employed and of the articles to be treated, inclusive of other external factors, such as atmospheric temperature, moisture, ventilation and the like, although the period of time extending from one to two days is enough under normal atmospheric conditions. Heat may be applied for accelerating the dry processing, but the application of heat is not essential in the present invention, because there is, as stated before, no need in the invention of decomposing the emulsifier by means of heating.

The objects of the present invention can also be materialized when the article to be treated is first wetted with an emulsion containing any of the aforespecified polysiloxanes in the order of concentration from 1 to 10 weight percent, and then the resultant article, after drying, is wetted with a solution containing zinc acetate or zinc formate and any of the aforespecified metallic compounds in the order of concentration from 1 to 10 percent by total metal weight, the range of concentration of the metallic compound employed in relation with zinc acetate or zinc formate being as specified before.

In order to provide a fuller understanding of the present invention, there are presented the following examples which are illustrative only, and in which spray rating was determined in association with the American Association of Textile Chemists and Colorists' standard test method:

#### Example 1

To 0.9 gram of benzylcetyltrimethylammonium chloride dissolved in a slight amount of water, there were added 90 grams of methylhydrogenpolysiloxane, and the mixture was dispersed with stirring for 5 minutes in 59.1 cc. of water to make up 150 grams of aqueous emulsion containing 60 weight percent of methylhydrogenpolysiloxane. The resultant emulsion was diluted with water to a concentration of 3 weight percent. There were then added with stirring zinc acetate and zirconium oxychloride in the order of respectively 10 percent and 0.2 percent by metal weight in relation to the polysiloxane weight present in the emulsion. In the resultant emulsion were dipped cotton poplin fabrics for about 30 minutes, squeezed to the order of about 2 times the original weight, and dried at room temperature ranging from 24° to 30° C. for 36 hours. Spray rating before and after washing was 100, and the treated fabrics exhibited an excellent good hand and soft touch.

The same results as stated above were obtained with 9 percent by metal weight of zinc formate employed in the place of aforesaid zinc acetate.

Almost the same results as stated above were also produced on the nylon, polyester and polyacrylonitrile fabrics treated in the same manners as described above.

#### Example 2

To a 3 percent methylhydrogenpolysiloxane emulsion prepared in accordance with the manners as described in Example 1, there were added with stirring zinc acetate and zinc stearate in the order of respectively 10 percent and 0.3 percent by metal weight in relation to the polysiloxane weight present in the emulsion. Cuprammonium rayon fabrics were then dipped in the resultant emulsion, squeezed and dried in the same manners as described in Example 1. Spray rating before and after washing was 100, producing an excellent good hand and agreeable soft touch.

#### Example 3

To a 3 percent aqueous methylhydrogenpolysiloxane emulsion prepared in accordance with the manners as described in Example 1, there were added with stirring zinc acetate and magnesium acetate in the order of respectively 7 percent and 3 percent by metal weight in relation to the polysiloxane weight present in the emulsion. The resultant emulsion was then applied to polyvinyl alcohol fabrics ("Vynylon," Kurashiki Rayon Kabushiki-kaisha, Osaka, Japan), and the treated articles were squeezed and dried in the same manners as described in Example 1. Spray rating before and after washing was 100, producing an excellent good hand and agreeable soft touch.

Almost the same results were obtained with zinc acetate and zirconyl acetate employed in the place of the aforespecified zinc acetate and magnesium acetate in the order of respectively 10 percent and 0.01 percent by metal weight, and with zinc acetate and tin acetate employed in the place of aforespecified zinc acetate and magnesium acetate in the order of 10 percent and 0.5 percent respectively by metal weight.

#### Example 4

To 3 percent methylhydrogenpolysiloxane emulsion prepared in accordance with the manners as described in Example 1, there were added with stirring zinc acetate and titanium oxide in the order of respectively 10 percent and 1 percent by metal weight in relation to the polysiloxane weight present in the emulsion. The resultant emulsion was then sprayed onto concrete pavements in the order of 1/m.<sup>2</sup>, and the pavements were allowed to dry for 48 hours at atmospheric temperature ranging from 24° to 33° C., producing a marked water-repellency as compared with non-treated pavements.

Almost the same water-repellency was obtained with any of zinc oxide, tin oxide and lead oxide employed in the order of 1 percent by metal weight in the place of the aforespecified titanium oxide.

#### Example 5

Cotton poplin fabrics were dipped for 30 minutes at room temperature in a 3 percent aqueous methylhydrogenpolysiloxane emulsion prepared in accordance with the manners as described in Example 1, squeezed to the order of about 2 times the original weight and dried at room temperature. The resultant fabrics were then dipped for 30 minutes at room temperature in an aqueous solution containing 5 percent of zinc acetate and 1 percent of sodium stearate by metal weight, squeezed to the order of about 2 times the weight of said fabrics, and dried at room temperature for 36 hours. Spray rating before and after washing was 100, exhibiting an excellent good hand and soft touch. All the room temperatures employed were from 24° to 30° C.

We claim:

1. A process for rendering articles water repellent comprising wetting the article to be treated with an aqueous emulsion containing 1 to 10 weight percent of a polysiloxane having a methyl hydrogen siloxane unit in the order of at least 50 weight percent, zinc acetate and zirconyl acetate, the quantity of zirconyl acetate employed being in the order of from  $\frac{1}{10,000}$  to  $\frac{1}{10}$  parts by weight

of zirconium in the zirconyl acetate per 1 part by weight of zinc in the zinc acetate, the total quantity of zinc acetate and zirconyl acetate being 1 to 15 percent by total metal weight in relation to the polysiloxane employed, and drying the wetted article at room temperature to provide said article with a water repellent finish resistant to washing.

2. A process for rendering articles water repellent comprising wetting the article to be treated with an aqueous emulsion containing 1 to 10 weight percent of a polysiloxane having a methyl hydrogen siloxane unit in the order of at least 50 weight percent, zinc acetate and tin acetate, the quantity of tin acetate employed being in the order of from  $\frac{1}{100}$  to  $\frac{1}{10}$  parts by weight of tin in the tin acetate per 1 part by weight of zinc in the zinc acetate, the total quantity of zinc acetate and tin acetate being 1 to 15 percent by total metal weight in relation to the polysiloxane employed, and drying the wetted article at room temperature to provide said article with a water repellent finish resistant to washing.

3. A process for rendering articles water repellent comprising wetting the article to be treated with an aqueous emulsion containing 1 to 10 weight percent of a polysiloxane having a methyl hydrogen siloxane unit in the order of at least 50 weight percent, zinc acetate and magnesium acetate, the quantity of magnesium acetate employed being in the order of from  $\frac{1}{10}$  to  $\frac{1}{2}$  parts by weight of magnesium in the magnesium acetate per 1 part by weight of zinc in the zinc acetate, the total quantity of zinc acetate and magnesium acetate being 1 to 15 percent by total metal weight in relation to the polysiloxane employed, and drying the wetted article at room temperature to provide said article with a water repellent finish resistant to washing.

4. A process for rendering articles water repellent comprising wetting the article to be treated with an aqueous emulsion containing 1 to 10 weight percent of a polysiloxane having a methyl hydrogen siloxane unit in the order of at least 50 weight percent, zinc acetate and zirconium oxychloride, the quantity of zirconium oxychloride employed being in the order of from  $\frac{1}{1,000}$  to  $\frac{1}{10}$  parts by weight of zirconium in the zirconium oxychloride per 1 part by weight of zinc in the zinc acetate, the total quantity of zinc acetate and zirconium oxychloride being 1 to 15 percent by total metal weight in relation to the poly-

siloxane employed, and drying the wetted article at room temperature to provide said article with a water repellent finish resistant to washing.

5. A process for rendering articles water repellent comprising wetting the article to be treated with an aqueous emulsion containing 1 to 10 weight percent of a polysiloxane having a methyl hydrogen siloxane unit in the order of at least 50 weight percent, zinc acetate and one stearate species selected from the group consisting of zinc stearate and sodium stearate, the quantity of said stearate species being in the order of from  $\frac{1}{1,000}$  to  $\frac{3}{10}$  parts by weight of metal of the respective stearate per 1 part by weight of zinc in the zinc acetate, the total quantity of zinc acetate and said stearate species being 1 to 15 percent by total metal weight in relation to the polysiloxane employed and drying the wetted article at room temperature to provide said article with a water repellent finish resistant to washing.

6. A process for rendering articles water repellent comprising wetting the article to be treated with an aqueous emulsion containing 1 to 10 weight percent of a polysiloxane having a methyl hydrogen siloxane unit in the order of at least 50 weight percent, zinc acetate and one oxide species selected from the group consisting of zinc oxide, titanium oxide, tin oxide and lead oxide, the quantity of said oxide species being in the order of  $\frac{1}{100}$  to  $\frac{1}{10}$  parts by weight of metal of the respective oxide, the total quantity of zinc acetate and said oxide species being 1 to 15 percent by total metal weight in relation to the polysiloxane employed and drying the wetted article at room temperature to provide said article with a water repellent finish resistant to washing.

#### References Cited

##### UNITED STATES PATENTS

|           |         |          |           |
|-----------|---------|----------|-----------|
| 2,386,259 | 10/1945 | Norton   | 117—123   |
| 2,588,367 | 3/1952  | Dennett  | 117—155 X |
| 2,588,393 | 3/1952  | Kauppi   | 260—18    |
| 2,645,629 | 7/1953  | Nitzsche | 117—161 X |
| 2,789,956 | 4/1957  | Eder     | 117—161 X |
| 2,934,519 | 4/1960  | Clark    | 117—161   |

WILLIAM D. MARTIN, *Primary Examiner.*

T. G. DAVIS, *Assistant Examiner.*